# EUROPEAN PATENT SPECIFICATION

(11) **EP 3 495 060 B1**
(45) Date of publication and mention of the grant of the patent: **24.08.2022**
(21) Application number: 18210547.8
(22) Date of filing: 05.12.2018
(51) Int. Cl.: B21D 22/20, B21D 22/28, B21D 51/26, B21D 22/30

(54) **METHOD OF PRODUCING CAN BODIES**
VERFAHREN ZUR HERSTELLUNG VON DOSENKÖRPERN
MÉTHODE DE PRODUCTION DES CORPS DE BOÎTES

(30) Priority: 05.12.2017 EP 17205572
(43) Date of publication of application: 12.06.2019
(73) Proprietor: Tata Steel IJmuiden B.V., 1951 JZ Velsen-Noord (NL)
(72) Inventor: JIMMINK, Alexander, 1970 CA IJmuiden (NL); KWAKKEL, Henri, 1970 CA IJmuiden (NL)
(74) Representative: Group Intellectual Property Services

(56) References cited:
- WO-A1-90/14179
- GB-A- 2 092 932
- US-A- 5 778 722
- US-A1- 2010 242 567
- US-B1- 6 634 203

## Description

### Field of the invention

This invention relates to an improved method of producing can bodies from a polymer coated metal substrate by the drawing and wall-ironing process.

### Background of the invention

The principle of draw- and wall ironing technology is well-known. The technology requires a circular blank for forming the (usually) cylindrical can body. The metal for the can bodies is usually supplied in coiled form. The coiled metal is uncoiled and blanks are stamped from the metal and produced into a so-called initial cup by a deep-drawing operation. This cup is deep drawn until no flanges are present. The cup is then redrawn in one or more redrawing steps to the final can diameter. In each redrawing step the maximum reduction of diameter is determined by the limiting drawing ratio, which is defined as the ratio of the maximum blank diameter that can be safely drawn into a cup without flange to the punch diameter. In any case the diameter of the initial cup is significantly larger than the diameter of the redrawn cup. In the final stage the thickness of the redrawn cup wall is reduced by wall-ironing the cup and produce a can body for a 2-piece can. This process involves pushing the redrawn cup through one or more ironing rings by means of a punch. The gap between the punch and the ironing ring determines the final thickness of the wall of the can body. For instance, a wall thickness of 0.30 mm in the redrawn cup may be reduced to 0.10 to 0.14 mm. Of course the height of the wall increases as a result.

After the DWI stage the edge of the can body has to be trimmed, because as a result of the inherent anisotropy of the metal the height of the can body is not the same everywhere on the circumference of the edge of the can body. This trimming also allows the final height of the can body to be tailored and prepared for the necking and flanging operation that is needed to receive the lid (the second piece of the two-piece can) after filling the can. Nowadays this lid is usually an easy open end, but it may also be a conventional lid which is to be opened by a can opener.

This type of can used to be made from tinplate. In order to be able to produce DWI cans from tinplate copious amounts of lubricants are needed, not only to 'cool away' the heat generated by the work-hardening of the material, but also to prevent tool surface wear and surface damage, and to provide a good can surface. Any swarf needs to be removed very thoroughly from the can body and therefore a very thorough washing is required. The copious amounts of lubricant and the need for a washing stage leads to the identification of the DWI-process as a 'wet DWI' process.

Recently alternative substrates have been developed for producing DWI can bodies: polymer coated metal sheet. This metal sheet, which may be aluminium sheet or steel sheet, can be produced as coiled metal and be provided with a polymer coating on one or both sides by film lamination or direct extrusion or the like.

This polymer coated metal sheet is suitable for producing can bodies by DWI and it is even possible to perform this with a minimum or even no lubricant. The polymer coating layer acts as lubricant. Also, because there is no exposed metal surface, there is also no risk of producing swarf, and therefore the need to wash the can bodies after the DWI-process is removed. Consequently this DWI process is referred to as a 'dry DWI' process.

Unfortunately, when producing can bodies from the polymer coated metal sheet there is a risk of formation of hairs at the edge of the can body, i.e. at the open end of the can body. As the polymer coating layer is softer than the metal substrate upon which the polymer coating layer is provided, the polymer coating layer deforms more easily than the metal substrate, and the polymer may be scraped off at the end. This manifests itself usually in the form or thread-like 'hairs'. If this happens then the DWI tooling may be polluted with hairs becoming dislodged from the edge, or the hairs may end up in the can body, and potentially in the cans contents when filled later, or exposes bare metal which might be hard enough to cause damage to the DWI-tooling. This is undesirable, and requires the can bodies to be rinsed, thus negating one of the advantages of the dry process.

US 6 634 203 B1 discloses a method for manufacturing a cylindrical can body from a polymer coated metal sheet comprising the steps of producing a circular blank from said polymer coated metal sheet, drawing an initial cup from said blank in a cupping step, redrawing said initial cup into a redrawn cup in a redraw step, wherein the redraw step comprises the following substeps:- positioning the initial cup in line with a cylindrical punch of a redraw apparatus;- clamping the circular bottom part of the initial cup between a ring-shaped redraw sleeve surrounding the punch and the redraw die thereby exerting a blank holder force on the bottom part of the initial cup;- pushing the punch through the hole in the redraw die, thereby reducing the diameter of the initial cup to form the redrawn cup; followed by- wall ironing said redrawn cup into a can body having its final height in a wall ironing step, wherein the wallironing is performed by using one or more one ironing rings in the wall ironing step, or- drawing the redrawn cup in a second redraw step to produce a can body having its final height.

### Objectives of the invention

It is the object of the invention to improve the production of can bodies from polymer coated metal sheet by the dry-DWI process in order to prevent the formation of hairs at the edge of the can body.

### Description of the invention

The object of the invention is reached by the method for manufacturing a cylindrical can body from a polymer coated metal sheet comprising the steps of producing a circular blank from said polymer coated metal sheet, drawing an initial cup from said blank in a cupping step, redrawing said initial cup into a redrawn cup in a redraw step, wherein the redraw step comprises the following successive substeps:
- positioning the initial cup in line with a cylindrical punch of a redraw apparatus;
- clamping the circular bottom part of the initial cup between a ring-shaped redraw sleeve surrounding the punch and the redraw die thereby exerting a blank holder force on the bottom part of the initial cup;
- pushing the punch through the hole in the redraw die, thereby reducing the diameter of the initial cup to form the redrawn cup and lifting the redraw sleeve, thereby removing the blank holder force, before the edge of the flange of the initial cup enters the operative part (OP) of the redraw die, thereby pushing the redrawn cup through
the redraw die without a blank holder force being exerted upon the flange; followed by
- wall ironing said redrawn cup into a can body having its final height in a wall ironing step, wherein the wall-ironing is performed by using one or more one ironing rings in the wall ironing step, or
- drawing the redrawn cup in a second redraw step to produce a can body having its final height.

Preferred embodiments are provided in the dependent claims.

The polymer coated metal sheet, which may be aluminium sheet or steel sheet, can be produced as coiled metal and is provided with a polymer coating on one or both sides. The polymer or polymer system comprising more than one layer of polymer on one side may differ from the one on the other side for reasons that the requirements for both sides differ, e.g. depending on the later use of the can body.

In this invention the blank holder force is reduced just before the edge of the initial cup enters the operative part (OP) of the redraw die by reducing the blank holder force (BHF) partly or completely on the redraw sleeve, or by effectively lifting the redraw sleeve from the edge of the initial cup. Preferably this lifting of the redraw sleeve is performed while the edge of the initial cup is less than 5 mm away from the OP. This ensures that the edge of the polymer coated metal is not pinched and this prevents the formation of hairs. Too early lifting is not preferred because the edges may wrinkle as a result. If the metal is very anisotrope, then the so-called ears may be too large to enable the timely lifting of the redraw sleeve to prevent pinching because the edge of one part of the circumference of the initial cup may have already entered the OP while the ears are still more than 5 mm removed from the OP. In that case the lifting of the redraw sleeve may be performed gradually to prevent pinching of the edge at the lowest part of the circumference of the cup and to prevent wrinkling of the ears. In any case the redraw sleeve must be lifted prior to the last part of the edge of the flange entering the operative part. It is clear that this process is more controlled the lower the anisotropy of the metal and benefits greatly from as isotrope a material as possible. The mechanical property associated with this is Δr which is defined as: $Δr = \frac{1}{2} ⋅ \left({r}_{0}-2⋅{r}_{45}+{r}_{90}\right)$ 0, 45 and 90 is the angle to the rolling direction of the tensile specimen taken from the metal sheet used as the substrate for the polymer coating and r is the ratio of the reduction in the width direction and the reduction in the thickness direction when measured during tensile testing.

### Brief description of the drawings

A schematic drawing of the set-up for redrawing an initial cup is provided in figure 1. The operative part of the redraw die as well as the operative part of the redraw sleeve are highlighted in figure 1 with the magnifying glass. These parts are depicted in more detail in figure 2a and 2b. The operative part is the part described by the radius R and delimited by the dashed lines. Preferably the angle over which the radius R angle is provided is 90°, i.e. the operative part is a quarter circle as seen in cross-section in figure 2a and 2b. For the sake of clarity it should be noted that the redraw die 2 as depicted in cross section in figure 1 is provided with a circular hole through which the initial cup 4 is pushed by a cylindrical punch 1 while being held to the flat area of the redraw die by the annular redraw sleeve 3. Figure 1 is schematic also in the sense that there is room between the cup, sleeve and redraw die, while in practice the redraw sleeve will push the initial cup onto the redraw die to prevent wrinkling

In an embodiment the radius of the OP and/or OPRS is reduced to a value of 2 to 6 x t, wherein t is the diameter of the material of the blank (or if the redraw step is performed more than one, t is the thickness of the bottom of the cup to be redrawn). Preferably at most 5 x t, more preferably at most 4 x t, even more preferably at most 3 x t or even at most 2,75 x t.

In this embodiment the decreased radius of the operative part of the redraw die R_{rd} or the radius of the operative part of the redraw sleeve Rᵣₛ allows to stretch-draw the polymer coated metal substrate. The reduction of the radius or radii is essential if the can body is required to have a certain height. Without the reduction of the radius or radii the polymer coated metal sheet would slip as a result of the reduced friction as compared with the same sheet with a metallic surface. To make it possible to stretchdraw the polymer coated metal sheet a degree of tension must be built up in the metal sheet i.e. during redrawing, and the building up of this tension is possible as a result of the reduced radius or radii. By preventing the slip by the increased friction as a result of the reduced radii the wall of the cup is elongated, in the area between the radii R_{rd} or Rᵣₛ, under the influence of the tensile force in the wall, thereby reducing the thickness of the wall and increasing the height of the can body.

The method according to the invention has the advantage that in comparison to conventional practice, where the emphasis of the elongation of the can wall is in the ironing stage, the elongation of the can wall by redrawing of the polymer coated redrawn cup takes place to a larger extent in the cupping stage and redrawing stage and to a lesser extent in the ironing stage.

The effect of the reduction of only the radius of the operative part of the redraw die or only of the radius of the operative part of the redraw sleeve is already very effective. By the reduction of radius of the operative part of both the redraw die and the redraw sleeve the maximum effect is reached, leading to the highest possible redrawn cup, which will then lead to the drawn and ironed can body with the largest possible wall height thereby allowing a reduced ironing step.

The reduced radius or radii of OP and/or OPRS has to be combined with a force imposed though the redraw sleeve upon the flange of the initial cup during the redraw step (this force is referred to as blank holder force or BHF, because the initial cup can be considered as a blank for the redrawing step). The redraw sleeve is cylindrical to achieve tension in the material as soon as possible during the redrawing. In conventional redraw processes the redraw sleeve is not cylindrical but tapered (see figure 3a).

In an embodiment the process according to the invention is performed with only one wall-ironing ring in the wall-ironing step. This process benefits from a maximum shift of deformation to the cupping and redrawing stage. The stretching of the wall of the initial cup during the redrawing step(s) is maximised, so that the only one wall-ironing ring is sufficient to finish the can body with the desired wall height. With the conventional methods the wall of the redrawn cup is not stretched to the same extent, or not at all, so that more reduction needs to be generated by the wall-ironing step, and this step then requires at least two rings. The use of one wall-ironing ring in combination with an increased elongation of the wall during the redrawing step(s) simplifies the wall-ironing process considerably thereby making it also more robust and easier to control in terms of temperature and deformation. The heat generated during the wall-ironing is also reduced if the wall-ironing reduction is smaller. In a dry-process, without external coolant, temperature control is especially important.

The radius R_{rd} or Rᵣₛ is expressed in terms of the initial thickness of the polymer coated metal sheet, which is also the thickness of the circular blank used to produce the initial cup from. The radius is at most 3 times the thickness of the polymer coated metal sheet or blank, preferably one radius or both radii is at most 2.75 times the thickness of the polymer coated metal sheet or blank, and more preferably at most 2.5 times. Even more preferably the radius or both radii is at most 2.25 or 2.0 times the thickness of the polymer coated metal sheet or blank. In an embodiment both R_{rd} and Rᵣₛ have the same value.

In an embodiment a burnishing step is provided by pushing the can body after the ironing operation through a burnishing ring. This relieves the tension in the can body wall and allows the can body to be stripped off easily.

The polymer coated steel substrates that can be processed by the process according to the invention are preferably based on polycondensates, such as polyesters, copolyesters (including PET, PBT, polyethylene furanoate (PEF), poly(lactic acid) (PLA)) or polyamides, polyolefins, elastomers, crystallisable polyaddition polymers, or any other polymer that can be formed in a film by extrusion. The polymer coating may consist of one or more layers. Preferably the polymer coating layer comprises or consists of polyethylene terephthalate, IPA-modified polyethylene terephthalate, CHDM-modified polyethylene terephthalate, polybutylene terephthalate, polyethylene naphthalate, polyethylene furanoate, poly (lactic acid) or copolymers or blends thereof.

The sheet metal preferably is tin coated steel sheet (tinplate), chromium-chromiumoxide coated steel sheet (ECCS), tinplate which was diffusion annealed to form an iron-tin alloy consisting of at least 80% of FeSn (50 at.% iron and 50 at.% tin) thereupon, or a chromium-chromiumoxide coated steel sheet produced by electroplating from a trivalent chromium electrolyte (such as TCCT^{®}).

The invention is also embodied in a can body produced by the method of the invention.

### Example

A 65 mm diameter can body is produced from 0.25 mm steel sheet with a polyester coating of 25 µm on both sides, leading to a total thickness t of 0.30 mm. The steel is a common extra low carbon (ELC) steel (see table 1). Blanks were produced therefrom and these were processed into initial cups. Using a redraw die with R_{rd} of 1.0 mm and of R_{rd} of 0.425 mm redraw cups were made in a single redraw step.

**Table 1: Composition of ELC-steel (in wt.%, bal. Fe and residual elements)**

| C | Mn | N | Alsol | P | S | B |
|---|---|---|---|---|---|---|
| 23 | 146 | 1.9 | 18 | 12 | 8 | 1.7 |

Wall thickness at 10 mm from bottom of redrawn cup (values including coating):
R_{rd} = 1.0 mm = 0.284 mm
R_{rd} = 0.425 mm = 0.238 mm

Wall thickness at mid height of the wall of the redrawn cup (values including coating):
R_{rd} = 1.0 mm = 0.275 mm
R_{rd} = 0.425 mm = 0.230 mm

The redrawn cup wall thickness is presented in figure 4. The height increases towards the top because of the material flow during deep drawing and the compressive forces in the material ion the circumference. This increased thickness is subsequently ironed 'out' in the subsequent ironing step. From figure 4 it can be seen that the height of the cup wall increases from 69 mm at R_{rd} 1 mm to 80 mm at R_{rd} of 0.425 mm, which is a 17% increase. This reduction is the result of the stretch-draw operation. In combination with one ironing ring an overall wall reduction of 50% can be reached. Lift off of the redraw sleeve was performed before the edge of the flange of the initial cup enters the operative part (OP) of the redraw die.

## Claims

1. Method for manufacturing a cylindrical can body from a polymer coated metal sheet comprising the steps of producing a circular blank from said polymer coated metal sheet, drawing an initial cup (4) from said blank in a cupping step, redrawing said initial cup into a redrawn cup in a redraw step, wherein the redraw step comprises the following substeps:
- positioning the initial cup (4) in line with a cylindrical punch (1) of a redraw apparatus;
- clamping the circular bottom part of the initial cup (4) between a ring-shaped redraw sleeve (3) surrounding the punch and the redraw die thereby exerting a blank holder force on the bottom part of the initial cup;
- pushing the punch (1) through the hole in the redraw die (2), thereby reducing the diameter of the initial cup to form the redrawn cup and lifting the redraw sleeve (3), thereby removing the blank holder force, before the edge of the flange of the initial cup (4) enters the operative part (OP) of the redraw die, thereby pushing the redrawn cup through the redraw die (2) without a blank holder force (BHF) being exerted upon the flange;
followed by
- wall ironing said redrawn cup into a can body having its final height in a wall ironing step, wherein the wall-ironing is performed by using one or more one ironing rings in the wall ironing step, or
- drawing the redrawn cup in a second redraw step to produce a can body having its final height.

2. Method according to claim 1 wherein the redraw sleeve (3) is lifted in the redraw step as soon as the edge of the flange of the initial cup (4) is still between 0.2 and 5.0 mm removed from the operative part (OP) of the redraw die (2).

3. Method according to claim 2 wherein the redraw sleeve (3) is lifted in the redraw step as soon as the edge of the flange of the initial cup (4) is still between 1.0 and 4.0 mm removed from the operative part (OP) of the redraw die (2).

4. Method according to any one of claims 1 to 3 wherein the redrawn cup is subjected to another redraw step by positioning the redrawn cup in line with a cylindrical punch of a redraw apparatus;
- clamping the circular bottom part of the redrawn cup between a ring-shaped redraw sleeve surrounding the punch and the redraw die thereby exerting a blank holder force on the bottom part of the redrawn cup;
- pushing the punch through the hole in the redraw die, thereby reducing the diameter of the redrawn cup to form the redrawn redrawn cup and lifting the redraw sleeve, thereby removing the blank holder force, before the edge of the flange of the initial cup enters the operative part (OP) of the redraw die, thereby pushing the redrawn redrawn cup through the redraw die without a blank holder force being exerted upon the flange;
followed by
- wall ironing said redrawn redrawn cup into a can body having its final height in a wall ironing step, wherein the wall-ironing is performed by using one or more one ironing rings in the wall ironing step, or
- drawing the redrawn redrawn cup in a third redraw step to produce a can body having its final height.

5. Method according to any one of claim 1 to 4 wherein the radius Rᵣₛ of the operative part of the redraw sleeve (OPRS) is between 2 to 6 x t, preferably at most 3 x t, wherein t is the thickness of the polymer coated metal sheet

6. Method according to claim 5 wherein the radius Rᵣₛ of the operative part of the redraw sleeve (OPRS) is at most 2.75 x t.

7. Method according to claim 5 wherein the radius Rᵣₛ of the operative part of the redraw sleeve (OPRS) is at most 2.5 x t.

8. Method according to any one of claim 1 to 7 wherein the radius R_{rd} of the operative part (OP) of the redraw die is between 2 to 6 x t, preferably at most 3 x t, wherein t is the thickness of the polymer coated metal sheet.

9. Method according to claim 8 wherein the radius of the operative part (OP) of the redraw die R_{rd} is at most 2.75 x t.

10. Method according to claim 8 wherein the radius R_{rd} of the operative part (OP) of the redraw die is at most 2.5 x t.

11. Method according to any one of the preceding claims wherein only one ironing ring is used.

12. Method according to any one of the preceding claims wherein a burnishing ring is used in addition to the drawing ring or drawing rings in the wall ironing step to remove tension in the can body thereby facilitating the stripping of the can body from the punch.

## Patentansprüche

1. Verfahren zum Herstellen eines zylindrischen Dosenkörpers aus einem polymerbeschichteten Metallblech, umfassend die Schritte des Produzierens eines kreisförmigen Rohlings aus dem polymerbeschichteten Metallblech, Ziehens eines Ausgangsbechers (4) aus dem Rohling in einem Tiefziehschritt, Nachziehens des Ausgangsbechers in einen nachgezogenen Becher in einem Nachziehschritt, wobei der Nachziehschritt die folgenden Unterschritte umfasst:
- Positionieren des Ausgangsbechers (4) in Linie mit einem zylindrischen Stempel (1) einer Nachziehvorrichtung;
- Klemmen des kreisförmigen unteren Teils des Ausgangsbechers (4) zwischen eine ringförmige Nachziehhülse (3), die den Stempel und die Nachziehmatrize umgibt, wodurch eine Rohlinghaltekraft auf den unteren Teil des Ausgangsbechers ausgeübt wird;
- Drücken des Stempels (1) durch das Loch in der Nachziehmatrize (2), wodurch der Durchmesser des Ausgangsbechers reduziert wird, um den nachgezogenen Becher zu bilden, und Anheben der Nachziehhülse (3), wodurch die Rohlinghaltekraft entfernt wird, bevor der Rand des Flansches des Ausgangsbechers (4) in den operativen Teil (OP) der Nachziehmatrize eintritt, wodurch der nachgezogene Becher durch die Nachziehmatrize (2) gedrückt wird, ohne dass eine Rohlinghaltekraft (BHF) auf den Flansch ausgeübt wird;
gefolgt von
- Wandabstrecken des nachgezogenen Bechers zu einem Dosenkörper, der seine finale Höhe aufweist, in einem Wandabstreckschritt, wobei das Wandabstrecken durch Verwenden von einem oder mehreren Abstreckringen in dem Wandabstreckschritt durchgeführt wird, oder
- Ziehen des nachgezogenen Bechers in einem zweiten Nachziehschritt, um einen Dosenkörper zu produzieren, der seine finale Höhe aufweist.

2. Verfahren nach Anspruch 1, wobei die Nachziehhülse (3) in dem Nachziehschritt angehoben wird, sobald der Rand des Flansches des Ausgangsbechers (4) noch zwischen 0,2 und 5,0 mm von dem operativen Teil (OP) der Nachziehmatrize (2) entfernt ist.

3. Verfahren nach Anspruch 2, wobei die Nachziehhülse (3) in dem Nachziehschritt angehoben wird, sobald der Rand des Flansches des Ausgangsbechers (4) noch zwischen 1,0 und 4,0 mm von dem operativen Teil (OP) der Nachziehmatrize (2) entfernt ist.

4. Verfahren nach einem der Ansprüche 1 bis 3, wobei der nachgezogene Becher einem weiteren Nachziehschritt unterzogen wird, indem der nachgezogene Becher in Linie mit einem zylindrischen Stempel einer Nachziehvorrichtung positioniert wird;
- Klemmen des kreisförmigen unteren Teils des nachgezogenen Bechers zwischen eine ringförmige Nachziehhülse, die den Stempel und die Nachziehmatrize umgibt, wodurch eine Rohlinghaltekraft auf den unteren Teil des nachgezogenen Bechers ausgeübt wird;
- Drücken des Stempels durch das Loch in der Nachziehmatrize, wodurch der Durchmesser des nachgezogenen Bechers reduziert wird, um den nachgezogenen nachgezogenen Becher zu bilden, und Anheben der Nachziehhülse, wodurch die Rohlinghaltekraft entfernt wird, bevor der Rand des Flansches des Ausgangsbechers in den operativen Teil (OP) der Nachziehmatrize eintritt, wodurch der nachgezogene nachgezogene Becher durch die Nachziehmatrize gedrückt wird, ohne dass eine Rohlinghaltekraft auf den Flansch ausgeübt wird;
gefolgt von
- Wandabstrecken des nachgezogenen nachgezogenen Bechers zu einem Dosenkörper, der seine finale Höhe aufweist, in einem Wandabstreckschritt, wobei das Wandabstreckziehen durch Verwenden von einem oder mehreren Abstreckringen in dem Wandabstreckschritt durchgeführt wird, oder
- Ziehen des nachgezogenen nachgezogenen Bechers in einem dritten Nachziehschritt, um einen Dosenkörper zu produzieren, der seine finale Höhe aufweist.

5. Verfahren nach einem der Ansprüche 1 bis 4, wobei der Radius Rᵣₛ des operativen Teils der Nachziehhülse (OPRS) zwischen 2 und 6 x t, bevorzugt höchstens 3 x t ist, wobei t die Dicke des polymerbeschichteten Metallblechs ist.

6. Verfahren nach Anspruch 5, wobei der Radius Rᵣₛ des operativen Teils der Nachziehhülse (OPRS) höchstens 2,75 x t ist.

7. Verfahren nach Anspruch 5, wobei der Radius Rᵣₛ des operativen Teils der Nachziehhülse (OPRS) höchstens 2,5 x t ist.

8. Verfahren nach einem der Ansprüche 1 bis 7, wobei der Radius R_{rd} des operativen Teils (OP) der Nachziehmatrize zwischen 2 und 6 x t, bevorzugt höchstens 3 x t ist, wobei t die Dicke des polymerbeschichteten Metallblechs ist.

9. Verfahren nach Anspruch 8, wobei der Radius des operativen Teils (OP) der Nachziehmatrize R_{rd} höchstens 2,75 x t ist.

10. Verfahren nach Anspruch 8, wobei der Radius R_{rd} des operativen Teils (OP) der Nachziehmatrize höchstens 2,5 x t ist.

11. Verfahren nach einem der vorhergehenden Ansprüche, wobei nur ein Abstreckring verwendet wird.

12. Verfahren nach einem der vorhergehenden Ansprüche, wobei ein Polierring zusätzlich zu dem Ziehring oder den Ziehringen in dem Wandabstreckschritt verwendet wird, um Spannung in dem Dosenkörper zu entfernen, wodurch das Abstreifen des Dosenkörpers von dem Stempel erleichtert wird.

## Revendications

1. Procédé permettant la fabrication d'un corps de boîte cylindrique à partir d'une tôle revêtue de polymère comprenant les étapes de production d'une ébauche circulaire à partir de ladite tôle revêtue de polymère, étirage d'une coupelle initiale (4) à partir de ladite ébauche dans une étape d'emboutissage, ré-étirage de ladite coupelle initiale en une coupelle ré-étirée dans une étape de ré-étirage, ladite étape de ré-étirage comprenant les sous-étapes suivantes :
- positionnement de la coupelle initiale (4) en ligne avec un poinçon cylindrique (1) d'un appareil de ré-étirage ;
- serrage de la partie inférieure circulaire de la coupelle initiale (4) entre un manchon de ré-étirage en forme d'anneau (3) entourant le poinçon et la matrice de ré-étirage exerçant ainsi une force de serre-flan sur la partie inférieure de la coupelle initiale ;
- poussée du poinçon (1) à travers le trou de la matrice de ré-étirage (2), réduisant ainsi le diamètre de la coupelle initiale pour former la coupelle ré-étirée et levage du manchon de ré-étirage (3), supprimant ainsi la force de serre-flan, avant que le bord de la bride de la coupelle initiale (4) ne pénètre dans la partie fonctionnelle (OP) de la matrice de ré-étirage, poussant ainsi la coupelle ré-étirée à travers la matrice de ré-étirage (2) sans qu'une force de serre-flan (BHF) soit exercée sur la bride ;
suivie par
- pressage-étirage de paroi de ladite coupelle ré-étirée en un corps de boîte possédant sa hauteur finale dans une étape de pressage-étirage de paroi, ledit pressage-étirage de paroi étant effectué à l'aide d'un ou plusieurs un anneaux de pressage-étirage dans l'étape de pressage-étirage de paroi, ou
- étirage de la coupelle ré-étirée dans une seconde étape de ré-étirage pour produire un corps de boîte possédant sa hauteur finale.

2. Procédé selon la revendication 1, ledit manchon de ré-étirage (3) étant soulevé lors de l'étape de ré-étirage dès que le bord de la bride de la coupelle initiale (4) est encore entre 0,2 et 5,0 mm éloigné de la partie fonctionnelle (OP) de la matrice de ré-étirage (2).

3. Procédé selon la revendication 2, ledit manchon de ré-étirage (3) étant soulevé lors de l'étape de ré-étirage dès que le bord de la bride de la coupelle initiale (4) est encore entre 1,0 et 4,0 mm éloigné de la partie fonctionnelle (OP) de la matrice de ré-étirage (2).

4. Procédé selon l'une quelconque des revendications 1 à 3, ladite coupelle ré-étirée étant soumise à une autre étape de ré-étirage par le positionnement de la coupelle ré-étirée en ligne avec un poinçon cylindrique d'un appareil de ré-étirage ;
- le serrage de la partie inférieure circulaire de la coupelle ré-étirée entre un manchon de ré-étirage en forme d'anneau entourant le poinçon et la matrice de ré-étirage, exerçant ainsi une force de serre-flan sur la partie inférieure de la coupelle ré-étirée ;
- la poussée du poinçon à travers le trou de la matrice de ré-étirage, réduisant ainsi le diamètre de la coupelle ré-étirée pour former la coupelle ré-étirée ré-étirée et le soulèvement du manchon de ré-étirage, supprimant ainsi la force de serre-flan, avant que le bord de la bride de la coupelle initiale n'entre dans la partie fonctionnelle (OP) de la matrice de ré-étirage, poussant ainsi la coupelle ré-étirée ré-étirée à travers la matrice de ré-étirage sans qu'une force de serre-flan ne soit exercée sur la bride ;
suivie par
- le pressage-étirage de paroi de ladite coupelle ré-étirée ré-étirée en un corps de boîte possédant sa hauteur finale dans une étape de pressage-étirage de paroi, ledit pressage-étirage de paroi étant effectué à l'aide d'un ou plusieurs un anneaux de pressage-étirage dans l'étape de pressage-étirage de paroi, ou
- l'étirage de la coupelle ré-étirée ré-étirée dans une troisième étape de ré-étirage pour produire un corps de boîte possédant sa hauteur finale.

5. Procédé selon l'une quelconque des revendications 1 à 4, ledit rayon Rᵣₛ de la partie fonctionnelle du manchon de ré-étirage (OPRS) étant compris entre 2 et 6 x t, de préférence au plus 3 x t, t étant l'épaisseur de la tôle revêtue de polymère.

6. Procédé selon la revendication 5, ledit rayon Rᵣₛ de la partie fonctionnelle du manchon de ré-étirage (OPRS) étant au plus de 2,75 x t.

7. Procédé selon la revendication 5, ledit rayon Rᵣₛ de la partie fonctionnelle du manchon de ré-étirage (OPRS) étant au plus de 2,5 x t.

8. Procédé selon l'une quelconque des revendications 1 à 7, ledit rayon R_{rd} de la partie fonctionnelle (OP) de la matrice de ré-étirage étant compris entre 2 et 6 x t, de préférence au plus 3 x t, t étant l'épaisseur de la tôle revêtue de polymère.

9. Procédé selon la revendication 8, ledit rayon de la partie fonctionnelle (OP) de la matrice de ré-étirage R_{rd} étant au plus de 2,75 x t.

10. Procédé selon la revendication 8, ledit rayon R_{rd} de la partie fonctionnelle (OP) de la matrice de ré-étirage étant au plus de 2,5 x t.

11. Procédé selon l'une quelconque des revendications précédentes, uniquement un anneau de pressage-étirage étant utilisé.

12. Procédé selon l'une quelconque des revendications précédentes, un anneau de brunissage étant utilisé en plus de l'anneau d'étirage ou des anneaux d'étirage dans l'étape de pressage-étirage de paroi pour supprimer la tension dans le corps de boîte facilitant ainsi le détachement du corps de boîte du poinçon.
